

# United States Patent

[19]

Pelzel et al.

[11] 3,772,007

[45] Nov. 13, 1973

[54] **WROUGHT ZINC ALLOY**

[75] Inventors: **Erich Pelzel**, Puchheim, near Munich; **Reiner Pelzel**, Munich-Lochhausen, both of Germany

[73] Assignee: **Metallgesellschaft AG**, Frankfurt am Main, Germany

[22] Filed: **Feb. 23, 1971**

[21] Appl. No.: **118,170**

3,006,758 10/1961 Giuliani et al. .... 75/178 R  
3,527,601 9/1970 Foerster ..... 75/178 C

## FOREIGN PATENTS OR APPLICATIONS

1,319,535 1/1963 France ..... 75/178 R

*Primary Examiner*—L. Dewayne Rutledge

*Assistant Examiner*—E. L. Weise

*Attorney*—Michael S. Striker

[30] **Foreign Application Priority Data**

Feb. 24, 1970 Germany ..... P 20 08 525.0

[52] **U.S. Cl.** ..... **75/178 A**, **75/178 AC**, **148/11.5**

[51] **Int. Cl.** ..... **C22c 17/00**

[58] **Field of Search** ..... **75/178 R**, **178 A**,  
**75/178 AC**, **178 AM**, **178 C**

[56] **References Cited**

### UNITED STATES PATENTS

2,428,959 10/1947 Boyle et al. ..... 75/178 R

[57]

## ABSTRACT

Wrought zinc alloy comprising 0.01 to 0.30% titanium, 0.01 to 2.00% manganese, 0.01 to 2.00% aluminum, balance zinc (99.9 to 99.99%).

The alloys have a high creep resistance, a high ductility and a high tensile strength.

**3 Claims, No Drawings**

## WROUGHT ZINC ALLOY

## BACKGROUND OF THE INVENTION

The invention relates to a zinc-titanium wrought alloy and a method of working it.

A wrought zinc alloy for sheets, strips, tubes, rods and wire, in addition to the requirement of adequate strength properties must also be suited for perfect cold working by folding, bending, pressure application and drawing. These properties are obtained in many of the wrought zinc alloys employed in industry.

It is for instance known (METALL 23 1969 issue 8, pages 782-785) that titanium-containing wrought zinc alloys with 0.05 to 0.5% titanium and 0.05 to 1.50% copper have a good creep resistance which reaches its maximum by hot working at temperatures of 150° to 300°C or cold working with subsequent hot working at temperatures between 150° and 300°C. The tensile strength in these cases increases with increasing copper contents from about 11 kp/mm<sup>2</sup> to 28 kp/mm<sup>2</sup> while at the same time the creep resistance increases from 6 kp/mm<sup>2</sup> to 9 kp/mm<sup>2</sup> and the residual elongation is limited to 1 percent per year. The increase of the creep resistance is principally obtained by a superfine grain due to the titanium contents. However, the increase in strength of the zinc alloy is undesirably associated with a strong increase of the elasticity. The resultant rebound therefore is an obstacle for a permanent set or deformation of the sheets or strips which are for instance shaped by machines to channel-formed members or tubes.

Furthermore, with an increase of the copper contents the cold brittleness of these zinc alloys increases fairly substantially. The formed sheets and strips therefore have a small ductility as can be determined by means of the folding test. For instance sheets and strips show indications of fracture at a direct folding by 180° at room temperature and below. A break-free folding by 180° is possible only if the wrought alloy is hot worked or cold worked with a subsequent heat treatment.

An improvement of the shapability of ductility at comparatively low temperatures is obtained if the copper content is limited to about 0.15 percent. In this case however there results a decrease of the tensile strength to 15 to 18 kp/mm<sup>2</sup>.

It is accordingly an object of the present invention to avoid these shortcomings and more specifically to provide for a zinc wrought alloy which has an optimum combination of creep resistance, plasticity or ductility and tensile strength.

## SUMMARY OF THE INVENTION

The invention resides in a titanium-containing wrought zinc alloy of the following composition:

0.01 to 0.30% titanium

0.01 to 2.00% manganese

balance zinc 99.9 to 99.99.

Preferably the manganese content is between 0.04 and 1.20 percent.

The invention also involves a process for improving the properties of the alloy by subjecting it to hot rolling at 120° to 350°C to the desired final dimensions or cold rolling to the final dimensions at temperatures between 20° and 120°C followed by aging for at least one hour at 120° to 350°C.

## DESCRIPTION OF THE INVENTION AND OF PREFERRED EMBODIMENTS

As indicated the preferred contents of manganese is 5 between 0.04 and 1.20 percent. Most preferred is the range between 0.10 and 0.80 percent.

It is also advantageous to include aluminum in the alloy in an amount between 0.005 and 0.80 percent.

Up to 50 percent of the titanium contents may be replaced by chromium. The total chromium content of the alloy however should not be in excess of 0.1 percent.

To obtain the maximum properties in the alloy of the invention there should not be present, as impurities, 15 more than 0.15 percent total content of copper and in no case more than up to 25 percent of the contents of manganese. Likewise the iron should not be in excess of 10 percent of the manganese contents and the maximum should be 0.03 percent.

Under normal circumstances adequate creep resistance is obtained for practical purposes. However, if it is desired to attain particularly high values it is advisable to subject the wrought alloy to hot rolling to final 25 dimensions at temperatures between 120° and 350°C or to subject it to cold rolling to final dimensions at temperatures between 20° and 120°C in which latter case the alloy should be aged for at least 1 hour at temperatures between 120° and 350°C. The heat treatments 30 suggested do not affect in any manner the other properties of the wrought alloy.

The following examples will further illustrate the invention. The alloys described in these examples were obtained by mixing in molten condition and were then 35 cast at 450°C to ingots of a thickness of 80 mm each. After solidification the ingots were cooled rolled in order to form sheets and strips of a thickness of 1 mm. The cold rolling was effected in several passes. Subsequent the elongation, tensile strength, creep resistance and foldability were determined to obtain a picture of the properties of the alloy.

## EXAMPLE 1

Zinc wrought alloy of the composition:

manganese 0.80%

titanium 0.15%

balance high-grade zinc 99.99%.

The properties of the alloy were as follows:

Elongation at break — > 40 percent

Tensile strength — 25 kp/mm<sup>2</sup>

Creep resistance — 10 kp/mm<sup>2</sup> at 1% elongation per year

Foldability — 180° without break

## EXAMPLE 2

Wrought zinc alloy of the composition:

manganese 0.40%

titanium 0.10%

aluminum 0.05%

balance high-grade zinc 99.99%.

The properties of the alloy were as follows:

Elongation at break — > 60 percent

Tensile strength — 20 kp/mm<sup>2</sup>

Creep resistance — 8 kp/mm<sup>2</sup> at 1 percent elongation per year

Foldability — 180° without break

## EXAMPLE 3

Wrought zinc alloy of the composition:  
 manganese 0.30%  
 titanium 0.03%  
 aluminum 0.70%  
 balance high-grade zinc 99.99%.

The properties of the alloy were as follows:  
 Elongation at break — > 100%  
 Tensile strength — 20 kp/mm<sup>2</sup>

Creep resistance — 4 kp/mm<sup>2</sup> at 1 percent elongation  
 per year  
 Foldability — 180° without break.

The accomplishments of the alloys of the invention are particularly in the features of a high ductility and high tear resistance along with a high creep resistance.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of this

invention and, therefore, such adaptations should and are intended to be comprehended within the meaning and range of equivalence of the following claims.

What is claimed as new and desired to be protected by Letters Patent is set forth in the appended

5 1. A wrought zinc alloy containing between 0.01 and 0.30% titanium, or chromium replacing a portion of the titanium in an amount up to 0.1 percent but not more than 50 percent of the titanium content, between 0.01 and 2.00% manganese, between 0.005 and 0.80% aluminum, copper in an amount up to 0.15 percent but not more than 25 percent of the manganese content, and iron in an amount up to 0.03 percent but not more than 10 percent of the manganese content, the balance of 10 the alloy being zinc.

2. A wrought zinc alloy containing 0.40% manganese, 0.10% titanium, 0.05% aluminum, and the balance of the alloy being zinc.

15 3. A wrought zinc alloy containing 0.30% manganese, 0.03% titanium, 0.70% aluminum, and the balance of the alloy being zinc.

\* \* \* \* \*

25

30

35

40

45

50

55

60

65